# EUROPEAN PATENT SPECIFICATION

(11) **EP 1 321 302 B1**
(45) Date of publication and mention of the grant of the patent: **05.08.2009**
(21) Application number: 02080095.9
(22) Date of filing: 09.12.2002
(51) Int. Cl.: B41M 5/00

(54) **inkjet recording element with porous organic particles**
Tintenstrahlaufzeichnungselement mit porösen organischen Teilchen
élément d'enregistrement par jet d'encre avec des particules organiques poreuses

(30) Priority: 20.12.2001 US 28130; 15.10.2002 US 271057
(43) Date of publication of application: 25.06.2003
(73) Proprietor: Eastman Kodak Company, Rochester NY 14650-2201 (US)
(72) Inventor: Landry-Coltrain, Christine J.T., Rochester, New York 14650-2201 (US); Leon, Jeffrey W., Rochester, New York 14650-2201 (US); Franklin, Linda M., Rochester, New York 14650-2201 (US); Yacobucci, Paul Daniel, Rochester, New York 14650-2201 (US)
(74) Representative: Derks, Wilbert

(56) References cited:
- EP-A- 0 802 245
- EP-A- 1 106 378
- JP-A- 07 137 433
- PATENT ABSTRACTS OF JAPAN vol. 014, no. 224 (M-0972), 11 May 1990 (1990-05-11) & JP 02 055186 A (CANON INC), 23 February 1990 (1990-02-23)

## Description

The invention relates to an inkjet recording element, more particularly to an inkjet recording element containing porous organic particles.

In a typical inkjet recording or printing system, ink droplets are ejected from a nozzle at high speed towards a recording element or medium to produce an image on the medium. The ink droplets, or recording liquid, generally comprise a recording agent, such as a dye or pigment, and a large amount of solvent The solvent, or carrier liquid, typically is made up of water, an organic material such as a monohydric alcohol, a polyhydric alcohol or mixtures thereof.

An inkjet recording element typically comprises a support having on at least one surface thereof an ink-receiving or image-forming layer and includes those intended for reflection viewing, which have an opaque support, and those intended for viewing by transmitted light, which have a transparent support.

An inkjet recording element that simultaneously provides an almost instantaneous ink dry time and good image quality is desirable. However, given the wide range of ink compositions and ink volumes that a recording element needs to accommodate, these requirements of inkjet recording media are difficult to achieve simultaneously.

Inkjet recording elements are known that employ porous or non-porous single layer or multilayer coatings that act as suitable ink receiving layers on one or both sides of a porous or non-porous support. Recording elements that use non-porous coatings typically have good image quality and stability but exhibit poor ink dry time. Recording elements that use porous coatings typically contain colloidal particulates and have poorer image stability but exhibit superior dry times.

While a wide variety of different types of porous image recording elements for use with inkjet printing are known, there are many unsolved problems in the art and many deficiencies in the known products which have severely limited their commercial usefulness. A major challenge in the design of a porous image-recording layer is to be able to obtain good quality, crack-free coatings. Inkjet prints, prepared by printing onto inkjet recording elements, are subject to environmental degradation. They are especially vulnerable to light fade and fade resulting from gaseous impurities in the air, such as ozone and nitrous oxide. Highly swellable hydrophilic layers can take an undesirably long time to dry, slowing printing speed. Porous layers speed the absorption of the ink vehicle, but often suffer from insufficient gloss and severe dye fade. Porous layers are also difficult to coat without cracking.

Japanese Kokai 07-137432 describes an inkjet paper having an ink-absorbing layer containing polyester resin particles with internal pores. However, there is a problem with this element in that the average particle size of the polyester resin is greater than 0.5 microns, and the element will have low surface gloss. The particles are made by an emulsification technique in which smaller resin particles are coalesced and fused into larger hollow particles.

EP 1 106 378 B1 discloses preparation of particles using a suspension technique to obtain hard, non-porous particles made from crosslinking acrylic polymers. The particles are neither porous nor ionic.

EP 0 802245 B1 discloses cationic acrylate ethylene oxide particles used as a swellable mordant. The polymerization and crosslinking of the particles are allowed to progress at the same time to grow particles."

It is an object of this invention to provide an inkjet recording element which will provide improved ink uptake speed. Another objective of the invention is to provide an inkjet recording element having high surface gloss. Another objective of the invention is to provide an inkjet recording element having a receiving layer that when printed upon has an excellent image quality and stability.

The present invention relates to an inkjet recording element comprising a support, at least one porous ink receiving layer comprising crosslinked porous polyester-containing particles having a mean diameter of less than 0.5 µm and having ionic groups, wherein said crosslinked porous polyester-containing particles are prepared from an unsaturated precursor condensation polymer that comprises polyester;
wherein the crosslinked porous polyester-containing particles are obtainable by crosslinking the unsaturated precursor condensation polymer within an oil-in-water emulsion in the presence of a water-immiscible organic solvent, wherein the crosslinking reaction is a radical initiated polymerization of an ethylenically unsaturated monomer which readily copolymerizes with the unsaturated units in the unsaturated precursor condensation polymer, after which the water-immiscible organic solvent is removed to yield the porous crosslinked polyester-containing particles in a dispersion.

The present invention also includes a method of forming an inkjet print comprising providing an inkjet recording element as described above and printing on said inkjet recording element utilizing an inkjet printer.

Using the invention, a recording element is obtained which will provide improved ink uptake speed, high surface gloss and, when printed upon, has an excellent image quality.

The present invention details the use of porous organic particles in an inkjet recording element, wherein the porous organic particles comprise an unsaturated condensation polymer reacted with a vinyl monomer. Porous, condensation polymer particles are obtainable by crosslinking an unsaturated precursor condensation polyester within an oil-in-water emulsion in the presence of a water-immiscible organic solvent. The crosslinked, porous condensation polymer particles may be prepared via methods which are analogous to those described below for porous polyester particles with the main difference being that an unsaturated precursor condensation polymer is used in lieu of an unsaturated precursor polyester. The precursor condensation polymer is a polymer containing a backbone consisting of repetitive organic diradicals linked together by an ester bond, or an ester bond and one or more of the following bond types: amide, carbonate, urethane, or urea bonds. The precursor condensation polymer contains ester bonds and preferably one or more of non-ester bond types. For example, the unsaturated condensation polymer may comprise at least one of ester-co-urethane, ester-co-urea, ester-co-amide, or ester-co-carbonate, most preferably ester-co-urethane or ester-co-carbonate. In one embodiment, the porous organic particles comprise an unsaturated condensation polymer reacted with a vinyl monomer such as styrene, divinylbenzene, divinyl adipate, and cyclohexanedimethanol divinyl ether. The polymer may be linear or branched.

The precursor condensation polymer may also contain chemical unsaturation through which it can be crosslinked within an oil-in-water emulsion in the presence of a water-immiscible organic liquid to afford porous particles. The chemical unsaturation may be present within the precursor polyester along the backbone, as functionalized end groups or as pendant groups. An example of the first case is a polyester-urethane of which one of the repetitive ester units is a maleate or fumarate moiety. An example of the second case is an alcohol-terminated polyurethane which has been reacted with methacryloyl chloride to afford methacrylate ester end groups. Preferably the chemical unsaturation will be present as backbone unsaturation.

The precursor condensation polymers may be synthesized using any of the techniques commonly known to those skilled in the art of polymer synthesis for preparing condensation polymers. In general, the methods involve the reaction of lewis acidic and lewis basic monomers, each with a functionalization number of two or more under solution or melt conditions. Specific reagent combinations are shown in Table 7. It should be noted that multifunctional reagents with functionality numbers other than 2 (for example, trifunctional, tetrafunctional) may also be used. Conditions may be chosen in which the different types of reagents will react in a single reactor. Alternately, a multiple stage approach may be used in which a prepolymer, macromonomer, or oligomer with appropriate terminating groups is reacted with one or more additional polyfunctional reagents in a subsequent step. For example, a polyester-carbonate may be prepared either by reacting a diacid chloride, a bischloroformate, and a diol in the same pot or by preparing a low molecular weight alcohol-terminated prepolymer, which is subsequently reacted with a bischloroformate.

**Table 7. Reagent combinations (difunctional cases) required for forming condensation polymers.**

| **Condensation polymer bond** | **Lewis acid** | **Lewis base** |
|---|---|---|
| Ester | Cyclic anhydride, diacid chloride, diester, diacid | Diol, diphenol |
| Urethane | Diisocyanate | Diol, diphenol |
| Urea | Diisocyanate, phosgene or derivative thereof | Diamine |
| Carbonate | Bischloroformate, phosgene or reactive derivative thereof | Diol, diphenol |
| Amide | Cyclic anhydride, diacid chloride, diester, diacid | Diamine |

The crosslinking reaction is a radical-initiated polymerization of an ethylenically unsaturated monomer which readily copolymerizes with the unsaturated units in the precursor condensation polymer. The precursor condensation polymer can be organic-soluble, in which case an added emulsifying agent may be necessary. In another embodiment of this method, the precursor condensation polymer can be water-soluble, water-dispersible, or amphiphilic in character, in which case the precursor condensation polymer acts as the emulsifying species and an added emulsifying agent is merely optional. The methods by which the porous condensation polymer particles may be prepared as well as the other reagents used in the preparation (i.e. emulsifiers, initiators, ethylenically unsaturated monomers, water-immiscible organic) are the same as those described below for the porous polyester particles. The porous, condensation polymer particles contain ionic groups, as described below for porous polyester particles. Preferably, these ionic groups will be quaternary ammonium moieties.

The porous, condensation polymer beads may have a mean diameter of 0.1 - 0.5 µm.

The most preferred porous organic particles useful for this invention are described in Serial Number 10/027,701 by Leon et al., (Docket 82842) entitled "Method of Preparation of Porous Polyester Particles". The crosslinked, porous polyester particles may be prepared by crosslinking an unsaturated precursor polyester within an oil-in-water emulsion in the presence of a water-immiscible organic solvent. A precursor polyester is a polyester containing unsaturated groups which is used in turn to make porous polyester particles. The crosslinking reaction is a radical-initiated polymerization of an ethylenically unsaturated monomer which readily copolymerizes with the unsaturated units in the precursor polyester. The precursor polyester can be organic-soluble, in which case an added emulsifying agent may be necessary. In another embodiment of this method, the precursor polyester can be water-soluble, water-dispersible, or amphiphilic in character, in which case the precursor polyester acts as the emulsifying species and an added emulsifying agent is merely optional. The water-immiscible organic solvent is removed to yield a dispersion of porous, crosslinked, polyester-containing particles.

The precursor polyesters which may be used to form the porous polyester particles useful for this invention may be branched or unbranched, contain chemical unsaturation, and may be soluble either in water-immiscible organic solvents or in water. Optionally, the precursor polyester may be self-emulsifying in water or amphiphilic or surfactant-like in character. The precursor polyesters may have any glass transition temperature, provided it fulfills the solubility requirements. Preferably, the number average molecular weight (Mn) is from 1,000 to 30,000 gm/mole.

As is well known in the art, polyesters are condensation products of polybasic acids or of corresponding acid equivalent derivatives such as esters, anhydrides or acid chlorides and polyhydric alcohols. It will be known that whenever "diacids" or "polyacids" are referred to in this document, that corresponding acid equivalent derivatives such as esters, anhydrides or acid chlorides are also included by reference. Polymerizable unsaturation may be introduced into the molecule by the selection of a polybasic acid or polyhydric alcohol, which contains α,β-ethylenic unsaturation. In most cases, the unsaturation will be contained within the polybasic acid unit. Optionally, one or more additional polyacids common in the art of polycondensation may be used in addition to the unsaturated polyacid. These ethylenically unsaturated polyacids include, but are not necessarily limited to maleic, fumaric, itaconic, phenylenediacrylic, citraconic and mesaconic acid. Other, additional polyacids which do not contain chemical unsaturation and can be used in polyesters are described in WO 01/00703. These diacids can include, but are not necessarily limited to malonic, succinic, glutaric, adipic, pimelic, azelaic, and sebacic acids, phthalic, isophthalic, terephthalic, tetrachlorophthalic, tetrahydrophthalic, trimellitic, trimesic, isomers of naphthalenedicarboxylic acid, chlorendic acid, trimellitic acid, trimesic acid, and pyromellitic acid.

Ethylenically unsaturated groups can also be introduced into the precursor polyester by synthetic modification. For example, a polyester with a high alcohol number can be reacted with an anhydride or acid chloride of acrylic acid or methacrylic acid in order to introduce ethylenically unsaturated units.

Precursor polyesters that may be suitable for this invention can furthermore be comprised of any of a wide variety of polyhydric alcohols which are well known in the art of polycondensation and may be aliphatic, alicyclic, or aralkyl. A description of suitable polyhydric alcohols is given in WO 01/00703. These alcohols can include, but are not necessarily limited to ethylene glycol, 1,3-propylene glycol, 1,6-hexanediol, 1,10-decanediol, 1,4-cyclohexanedimethanol, 1,4-cyclohexanediol, hydroquinone bis (hydroxyethyl) ether, diethylene glycol, neopentyl glycol, bisphenols such as bisphenol A, ethylene oxide and propylene oxide adducts of bisphenol A, pentaerythritol, trimethylolpropane, and polyester polyols, such as that obtained by the ring-opening polymerization of ε-caprolactone. Additionally, A-B type polycondensation monomers which contain both hydroxyl and acid derivative functions can be used as well as monoacids and monoalcohols.

In one embodiment of this invention, precursor polyesters which are water-soluble, surfactant-like, or self-emulsifying and additionally contain chemical unsaturation may be utilized. Water-soluble, surfactant-like, and self-emulsifying polyesters are well known in the art and may contain one or more type of hydrophilic chemical group, functionality, or monomer, such as carboxylate, quaternary ammonium, sulfonate, sulfate, sulfonium, phosphonium, iminosulfonyl, or polymeric or oligomeric oxyethylene segments. Precursor polyesters used to form the porous polyester particles useful in this invention may additionally contain one or more polyacid or polyol monomers which contain ethylenic unsaturation as detailed above. The water-soluble, surfactant-like, and self-emulsifying precursor polyesters used to form the porous polyester particles useful in this invention may contain one or more diacid or diol components which can induce hydrophilic character or water-solubility. The most common hydrophilic diol used for this purpose is polyethylene glycol. Additionally, tertiary amine units substituted with two or three hydroxyalkyl groups can be incorporated within a precursor polyester and rendered ionic either by quaternization with an alkylating agent or by neutralization with an acid. A commonly used class of diacid components used to impart hydrophilicity to polyesters includes compounds containing sulfonate or sulfonimide salts. Some suitable sulfonated diacids are described in U.S. patents 4,973,656 and 5,218,042. Examples of such diacids are 5-sodiosulfoisophthalic acid, 2-sodiosulfobutanoic acid, and di-Me sodioiminobis(sulfonyl-*m*-benzoate). Another common strategy for the hydrophilization of polyesters involves the neutralization of the acid end groups of polyester with a relatively high acid number. Preferably, the acid number is at least 10. Most preferably the acid number is greater than 25. The neutralization agent is usually an alkali metal hydroxide or an amine. Polyesters containing ethylenic unsaturation and neutralized acid end groups can also be used in this invention. In the preferred case, the unsaturated precursor polyester will contain an ionic group equivalent weight of from 400 to 2000 grams of polymer per mole of ionic unit.

The ethylenically unsaturated monomers useful for crosslinking the precursor polyesters in this invention may be monomers commonly used in the art of addition polymerization. These include, but are not necessarily limited to methacrylic acid esters, such as methyl methacrylate, ethyl methacrylate, isobutyl methacrylate, 2-ethylhexyl methacrylate, benzyl methacrylate, phenoxyethyl methacrylate, cyclohexyl methacrylate and glycidyl methacrylate, acrylate esters such as methyl acrylate, ethyl acrylate, isobutyl acrylate, 2-ethylhexyl acrylate, benzyl methacrylate, phenoxyethyl acrylate, cyclohexyl acrylate, and glycidyl acrylate, styrenics such as styrene, α-methylstyrene, 3- and 4-chloromethylstyrene, halogen-substituted styrenes, and alkyl-substituted styrenes, vinyl halides and vinylidene halides, N-alkylated acrylamides and methacrylamides, vinyl esters such as vinyl acetate and vinyl benzoate, vinyl ethers, such as butyl vinyl ether and cycloxexanedimethanol divinyl ether, allyl alcohol and its ethers and esters, and unsaturated ketones and aldehydes such as acrolein and methyl vinyl ketone and acrylonitrile.

In addition, small amounts (typically less than 10% of the total weight of the polymerizeable solids) of one or more water-soluble ethylenically unsaturated monomer can be used. Such monomers include but are not necessarily limited to styrenics, acrylates, and methacrylates substituted with highly polar groups, unsaturated carbon and heteroatom acids such as acrylic acid, methacrylic acid, fumaric acid, maleic acid, itaconic acid, vinylsulfonic acid, vinylphosphonic acid, and their salts, vinylcarbazole, vinylimidazole, vinylpyrrolidone, and vinylpyridines.

Especially useful in this invention are monomers containing more than one ethylenically unsaturated unit, such as trimethylolpropane triacrylate, ethylene glycol dimethacrylate, isomers of divinylbenzene, divinyl adipate, cyclohexanedimethanol divinyl ether and ethylene glycol divinyl ether.

Ethylenically unsaturated monomers which are preferred for this invention are styrenics, vinyl ethers, and methacrylates. Divinylbenzene (m, and p isomers), styrene, divinyl adipate, and ethylene glycol dimethacrylate are especially preferred.

Any of the common water-soluble or organic-soluble free radical polymerization initiators known in the art of addition polymerization can be used for this invention. These include, but are not restricted to azo compounds, such as 2,2'-azobis(4-methoxy-2,4-dimethylvaleronitrile), (1-pheneylethyl)azodiphenylmethane, 2-2'-azoisobutyronitrile (AIBN), 1,1'-azobis(1-cyclohexanedicarbonitrile), 4,4'-azobis(4-cyanopentanoic acid), and 2,2'-azobis(2-amidinopropane) dihydrochloride, organic peroxides, organic hydroperoxides, peresters, and peracids such as benzoyl peroxide, lauryl peroxide, capryl peroxide, acetyl peroxide, t-butyl hydroperoxide, t-butyl perbenzoate, cumyl hydroperoxide, peracetic acid, 2,5-dimethyl-2,5-di(peroxybenzoate), and p-chlorobenzoly peroxide, persulfate salts such as potassium, sodium and ammonium persulfate, disulfides, tetrazenes, and redox initiator systems such as H₂O₂/Fe²⁺, persulfate/bisulfite, oxalic acid/Mn³⁺, thiourea/Fe³⁺, and benzoyl perozide/dimethylaniline.

Optionally, a small amount of a cosurfactant stabilizer, typically comprising 1-10% by weight of the organic phase, may be added to the organic phase of this invention. These hydrophobic compounds are known to prevent Ostwald ripening in certain types of emulsion and suspension polymerization. Excellent discussions of cosurfactants are given in Emulsion Polymerization and Emulsion Polymers by Peter A Lovell and Mohammed S. El-Aaser, (John Wiley and Sons: Chichester, 1997; pp. 700-721) and US Patent 5,858,634. The most common cosurfactants are hexadecane and hexadecanol. Other useful cosurfactants may also serve other roles, such as acting as monomers or initiators. An example of the former is lauryl methacrylate. An example of the latter is lauroyl peroxide.

If a precursor polyester is used in this invention which is not soluble or dispersible in water, then an emulsifier may additionally be used, although an emulsifier can be used in tandem with a water-soluble or water-dispersible precursor polyester. It may be preferable that the emulsifier be present in the aqueous phase. Though a very large variety of emulsifiers are known in the art, most of these fit into the three basic categories of surfactants, colloidal inorganics, and protective colloids. There exist a tremendous number of known surfactants. Good reference sources for surfactants are the *Surfactant Handbook* ( GPO: Washington, D. C., 1971) and *McCutcheon's Emulsifiers and Detergents* (Manufacturing Confectioner Publishing Company: Glen Rock, 1992). There are no general restrictions for the surfactants which may be useful in this invention. Useful surfactants can be anionic, cationic, zwitterionic, neutral, low molecular weight, macromolecular, synthetic, or extracted or derived from natural sources. Some examples include, but are not necessarily limited to: sodium dodecylsulfate, sodium dodecylbenzenesulfonate, sulfosuccinate esters, such as those sold under the AEROSOL^{®} trade name, flourosurfactants, such as those sold under the ZONYL^{®} and FLUORAD^{®} trade names, ethoxylated alkylphenols, such as TRITON^{®} X-100 and TRITON^{®} X-705, ethoxylated alkylphenol sulfates, such as RHODAPEX^{®} CO-436, phosphate ester surfactants such as GAFAC® RE-90, hexadecyltrimethylammonium bromide, polyoxyethylenated long-chain amines and their quaternized derivatives, ethoxylated silicones, alkanolamine condensates, polyethylene oxide-co-polypropylene oxide block copolymers, such as those sold under the PLURONIC^{®} and TECTRONIC^{®} trade names, N-alkylbetaines, N-alkyl amine oxides, and fluorocarbon-poly(ethylene oxide) block surfactants, such as FLUORAD^{®} FC-430.

Protective colloids useful in this invention include, but are not necessarily limited to: poly (ethylene oxide), hydroxyethyl cellulose, poly (vinyl alcohol), poly (vinyl pyrrolidone), polyacrylamides, polymethacrylamides, sulfonated polystyrenes, alginates, carboxy methyl cellulose, polymers and copolymers of dimethylaminoethylmethacrylate, water soluble complex resinous amine condensation products of ethylene oxide, urea and formaldehyde, polyethyleneimine, casein, gelatin, albumin, gluten and xanthan gum. Protective colloids are a class of emulsifiers which may be used in lieu of or in addition to a surfactant. They may be typically dissolved or dispersed in the aqueous phase prior to the emulsification step.

Similarly, colloidal inorganic particles can be employed as emulsifiers as part of a limited coalescence process. Colloidal inorganic particles can be employed in lieu of or in addition to any other type of emulsifier listed, such as a surfactant or protective colloid. They may be also added to the aqueous phase. Limited coalescence techniques have been describe in numerous patents such as U.S. Patents 4,833,060 and 4,965,131. A colloidal inorganic which is particularly useful in this invention is LUDOX^{®} TM sold by Du Pont.

Additional additives which can be incorporated into the porous organic particles useful in this invention include pigments, dyes, biocides, fungicides, electrolytes, buffers, UV-absorbers, antioxidants and chain transfer agents.

The porous polyester particles useful for this invention comprise porous polyester particles having a mean diameter of less than 0.5 µm. For optimal ink absorption properties and coating quality, it may be preferable that the porous polyester particles have a mean diameter range from 0.1 to less than 0.5 µm, and more preferably, that the porous polyester particles have a mean diameter range from 0.2 to 0.3 µm. The diameter of the particles can be measured by any method known in the art. One such method may be laser light scattering of dilute dispersions of the particles, using a commercially available instrument such as the Horiba LA-920, manufactured by Horiba LTD. Typically, a sample of porous polyester particles will contain a population of particles having a distribution of sizes. This is the particle size distribution, and is characterized by a mean diameter, a standard deviation, and a coefficient of variation. The mathematical equations defining these terms can be found in any basic text on statistical analysis, such as "Principles of Instrumental Analysis, 4th Edition", by D. A. Skoog and J. J. Leary, Harcourt Brace College Publishers, Orlando, FL, 1971 (Appendix A-6). The mean diameter is the arithmetic mean of the particle size distribution. The coefficient of variation (CV) of a distribution is the ratio of the standard deviation of the distribution to the mean diameter, given as a percent. The porous polyester particles useful for this invention can have a relatively large distribution of particle sizes within one mode, and the standard deviation in the mean diameter can be from 0.3 times the mean particle diameter to 3 times the mean particle diameter. In a system of particles, there can be a single mode or peak to this distribution of sizes, or there can be several modes, each mode being characterized by a mean diameter, a standard deviation, and a coefficient of variation. For example, the porous polyester particles can be a system composed of particles having a mode with a mean diameter of less than 0.5 µm and particles having a mode with mean diameter greater than 0.5 µm, preferably having a mean diameter from 1 to 10 µm, and most preferably having a mean diameter from 1 to 3 µm. The relative proportions of these two modes are calculated from the relative areas under the curves representing the modes, and should add up to 100 %.

As discussed above, the porous polyester particles contain ionic groups. Preferably the particles will have an ionic group equivalent weight of from 40 to 2000 grams per mole of ionic unit. These ionic groups may be ammonium (primary, secondary, tertiary, or quaternary), pyridinium, imidazolium, alkylsulfonates, alkylthiosulfate, carboxylate, phosphonium or sulfonium. Copolymerizable, α, β-ethylenically unsaturated monomers containing a preformed ionic functionality can be used in any of the polymerization processes described herein. Suitable monomers which can be used include, for example, the following monomers and their mixtures: cationic ethylenically unsaturated monomers, for example, vinylbenzyltrimethylammonium chloride, vinylbenzyldimethyl-dodecylammonium chloride, other vinylbenzylammonium salts in which the three other ligands on the nitrogen can be any alkyl or carbocyclic group including cyclic amines such as piperidine, the counter ions of which can be halides, sulfonates, phosphates, sulfates, [2-(methacryloyloxy)ethyl]trimethyl-ammonium chloride, [2-(acryloyloxy)ethyl]-trimethylammonium p-toluene-sulfonate, and other acrylate and methacrylate ammonium salts in which the alkyl group connecting the acrylic function to the nitrogen can be ≥ 2 carbon atoms long and the other three nitrogen ligands can be any alkyl or carbocyclic group including cyclic amines such as piperidine, and benzyl, 4-vinyl-1-methylpyridinium methyl sulfate, 3-methyl-1-vinylimidazolium methosulfate, and other vinylpyridinium and vinylimidazolium salts in which the other nitrogen ligand may be any alkyl or cycloalkyl group, vinyltriphenylphosphonium bromide, vinylbenzyltriphenylphosphonium tosylate, and other phosphonium salts in which the other three phosphorous ligands may be any aromatic or alkyl group. In a preferred embodiment, the cationic functionality may be vinylbenzyltrimethylammonium chloride, vinylbenzyl-N-butylimidazolium chloride, vinylbenzyldimethyldodecylammonium chloride or vinylbenzyl-dimethyloctadecylammonium chloride.

Other suitable copolymerizable, α, β-ethylenically unsaturated monomers containing a preformed ionic functionality which can be used include, for example, the following monomers and their mixtures: anionic ethylenically unsaturated monomers such as 2-phosphatoethyl acrylate potassium salt, 3-phosphatopropyl methacrylate ammonium salt, and other acrylic and methacrylic esters of alkylphosphonates in which the alkyl group connecting the acrylic function to the phosphate function can be ≥ 2 carbon atoms long, the counter ions of which can be alkali metal cations, quaternary ammonium cations, phosphonium cations, or the like, sodium methacrylate, potassium acrylate, and other salts of carboxylic acids, styrenesulfonic acid ammonium salt, methyltriphenylphosphonium styrenesulfonate, and other styrene sulfonic acid salts, 2-sulfoethyl methacrylate pyridinium salt, 3-sulfopropyl acrylate lithium salt, and other acrylic and methacrylic esters of alkylsulfonates, and other sulfonates such as ethylene sulfonic acid sodium salt. In a preferred embodiment, the anionic functionality may be trimethylamine hydrochloride salt of methacrylic acid, dimethylbenzylamine hydrochloride salt of methacrylic acid, dimethyldodecyl-amine hydrochloride salt of methacrylic acid or methyltrioctylammonium salt of styrenesulfonic acid.

The ionic group can also be formed after the polymer particle is prepared by modifying non-ionic monomers to make them (or part of them) ionic. All of the cationic and anionic functionalities mentioned above can be incorporated by modifying a non-ionic polymer particle.

The product particles, having excellent colloidal stability, can be stored as an aqueous dispersion or freeze dried to yield a solid powder comprising dry particles which will easily redisperse in water.

The ink receiving layer of the inkjet recording element may be formed by coating a mixture comprised of these porous organic particles and a binder in an amount insufficient to alter the porosity of the porous receiving layer onto a support, and then drying to remove approximately all of the volatile components. In a preferred embodiment, the polymeric binder is a hydrophilic polymer such as polyvinylpyrrolidone and vinylpyrrolidone-containing copolymers, polyethyloxazoline and oxazoline-containing copolymers, imidazole-containing polymers, polyacrylamides and acrylamide-containing copolymers, poly(vinyl alcohol) and vinyl-alcohol-containing copolymers, poly(vinyl methyl ether), poly(vinyl ethyl ether), poly(alkylene oxides), gelatin, cellulose ethers, poly(vinylacetamides), partially hydrolyzed poly(vinyl acetate/vinyl alcohol), poly(acrylic acid), sulfonated or phosphated polyesters and polystyrenes, casein, albumin, chitin, chitosan, dextran, pectin, collagen derivatives, collodian, agar-agar, arrowroot, guar, carrageenan, tragacanth, xanthan, rhamsan. In another preferred embodiment of the invention, the hydrophilic polymer is hydroxyethyl cellulose, hydroxypropyl cellulose, hydroxypropyl methyl cellulose, methyl cellulose, or a poly(alkylene oxide). In still another preferred embodiment, the polymeric binder may be a latex such as poly(styrene-co-butadiene), polyurethane, polyester, poly(acrylate), poly(methacrylate), a copolymer of n-butylacrylate and ethylacrylate, and a copolymer of vinylacetate and n-butylacrylate. In still another preferred embodiment, the polymeric binder may be a water dispersible condensation polymer such as a polyurethane. In still another preferred embodiment, the binder may be a condensate of alkoxysilanes or other metal sols such as alumina sol, titania sol, or zirconia sol. Mixtures of the above listed hydrophilic polymers can be used. The binder should be chosen so that it is compatible with the aforementioned particles.

The amount of polymer binder used should be sufficient to impart cohesive strength to the inkjet recording element, but should also be minimized so that the interconnected pore structure formed by the aggregates is not filled in by the binder. In a preferred embodiment of the invention, the porous organic particles are present in an amount of from 50 to 95 % by weight, and most preferably, in an amount from 75 to 90 % by weight of the layer.

Since the image recording element may come in contact with other image recording articles or the drive or transport mechanisms of image recording devices, additives such as filler particles, surfactants, lubricants, crosslinking agents, matte particles may be added to the element to the extent that they do not degrade the properties of interest.

Filler particles may be used in the ink receiving layer such as silicon oxide, fumed silica, silicon oxide dispersions such as those available from Nissan Chemical Industries and DuPont Corp., aluminum oxide, fumed alumina, calcium carbonate, barium sulfate, barium sulfate mixtures with zinc sulfide, inorganic powders such as γ-aluminum oxide, chromium oxide, iron oxide, tin oxide, doped tin oxide, alumino-silicate, titanium dioxide, silicon carbide, titanium carbide, and diamond in fine powder, as described in U.S. Patent 5,432,050.

A dispersing agent, or wetting agent can be present to facilitate the dispersion of the filler particles. This helps to minimize the agglomeration of the particles. Useful dispersing agents include, but are not limited to, fatty acid amines and commercially available wetting agents such as Solsperse® sold by Zeneca, Inc. (ICI). Preferred filler particles may be silicon oxide, aluminum oxide, calcium carbonate, and barium sulfate. Preferably, these filler particles have a median diameter less than 1.0 µm. The filler particles can be present in the amount from 0 to 80 percent of the total solids in the dried ink receiving layer, most preferably in the amount from 0 to 40 percent.

In order to obtain adequate coatability, rheology modifiers known to those familiar with such art such as thickening agents or polymers may be used. These include associative thickeners such as hydrophobically modified hydroxyethylcellulose, hydrophobically modified alkali-soluble or alkali swellable emulsions, and hydrophobically modified ethylene oxide urethane block copolymers such as those supplied by Rohm & Haas under the trade name of Acusol ® and Dow Chemical under the trade name of Polyphobe®, and non-associative thickeners such as hydroxyethyl cellulose, hydroxypropyl methyl cellulose, sodium carboxy methyl cellulose, xanthan gum, guargum, and carrageenan.

The ink jet recording element may include lubricating agents. Lubricants and waxes useful either in the ink receiving layer or on the side of the element that is opposite the ink receiving layer include, but are not limited to, polyethylenes, silicone waxes, natural waxes such as carnauba, polytetrafluoroethylene, fluorinated ethylene propylene, silicone oils such as polydimethylsiloxane, fluorinated silicones, functionalized silicones, stearates, polyvinylstearate, fatty acid salts, and perfluoroethers. Aqueous or non-aqueous dispersions of submicron size wax particles such as those offered commercially as dispersions of polyolefins, polypropylene, polyethylene, high density polyethylene, microcrystalline wax, paraffin, natural waxes such as carnauba wax, and synthetic waxes from such companies as, but not limited to, Chemical Corporation of America (Chemcor), Inc., Michelman Inc., Shamrock Technologies Inc., and Daniel Products Company, are useful.

In order to obtain adequate coatability, additives known to those familiar with such art such as surfactants, defoamers, alcohol may be used. Coating aids and surfactants include, but are not limited to, nonionic fluorinated alkyl esters such as FC-430®, FC-431®, FC-10®, FC-171® sold by Minnesota Mining and Manufacturing Co., Zonyl® fluorochemicals such as Zonyl-FSN®, Zonyl-FTS®, Zonyl-TBS®, Zonyl-BA® sold by DuPont Corp., other fluorinated polymer or copolymers such as Modiper F600® sold by NOF Corporation, polysiloxanes such as Dow Coming DC 1248®, DC200®, DC510®, DC 190® and BYK 320®, BYK 322®, sold by BYK Chemie and SF 1079®, SF1023®, SF 1054®, and SF 1080® sold by General Electric, and the Silwet® polymers sold by Union Carbide, polyoxyethylene-lauryl ether surfactants, sorbitan laurate, palmitate and stearates such as Span® surfactants sold by Aldrich, poly(oxyethylene-co-oxypropylene) surfactants such as the Pluronic® family sold by BASF, and other polyoxyethylene-containing surfactants such as the Triton X® family sold by Union Carbide, ionic surfactants, such as the Alkanol® series sold by DuPont Corp., and the Dowfax® family sold by Dow Chemical. Specific examples are described in MCCUTCHEON's Volume 1: Emulsifiers and Detergents, 1995, North American Edition.

The ink receiving layer may include crosslinking agents. Any crosslinking agent may be used provided its reactive functionalities have the appropriate reactivity with specific chemical units in the binder. Some common crosslinkers which can crosslink binders rich in lewis basic functionalities include, but are not necessarily limited to: carbodiimides, polyvalent metal cations, organic isocyanates such as tetramethylene diisocyanate, hexamethylene diisocyanate, diisocyanato dimethylcyclohexane, dicyclohexylmethane diisocyanate, isophorone diisocyanate, dimethylbenzene diisocyanate, methylcyclohexylene diisocyanate, lysine diisocyanate, tolylene diisocyanate, diphenylmethane diisocyanate, aziridines such as taught in U. S. Patent 4,225,665, ethyleneimines such as Xama-7® sold by EIT Industries, blocked isocyanates such as CA BI-12 sold by Cytec Industries, melamines such as methoxymethylmelamine as taught in U. S. Patent 5,198,499, alkoxysilane coupling agents including those with epoxy, amine, hydroxyl, isocyanate, or vinyl functionality, Cymel® crosslinking agents such as Cymel 300®, Cymel 303®, Cymel 1170®, Cymel 1171® sold by Cytec Industries, and bis-epoxides such as the Epon® family sold by Shell. Other crosslinking agents include compounds such as aryloylureas, aldehydes, dialdehydes and blocked dialdehydes, chlorotriazines, carbamoyl pyridiniums, pyridinium ethers, formamidinium ethers, vinyl sulfones, boric acid, dihydroxydioxane, and polyfunctional aziridines such as CX-100 (manufactured by Zeneca Resins). Such crosslinking agents can be low molecular weight compounds or polymers, as discussed in U. S. Patent 4,161,407 and references cited.

To improve colorant fade, UV absorbers, radical quenchers or antioxidants may also be added to the ink-receiving layer as is well known in the art. Examples include polyalkylenepolyamine-dicyanodiamide based polycondensation products, water soluble reducing agents, such as sulfites, nitrites, phosphates, thiosulfates, ascorbic acid or salts thereof, hydroxylamine derivatives, and glucose, sulfur-containing compounds, such as thiocyanates, thiourea, 2-mercaptobenzimidazole, 2-mercaptobenzthiazole, 2-mercaptobenzoxazole, 5-mercapto-1-methyl-tetrazole, 2,5-dimercapto-1,3,4-triazole, 2,4,6-trimercaptocyanuric acid, thiosalicylic acid, thiouracil, 1,2-bis(2-hydroxyethylthio)ethane, or hydrophobic antioxidant emulsified dispersions, such as hindered phenol based antioxidants, piperidine based antioxidants or hindered amines. UV absorbers include those described in Japanese Patent Publication Open to Public Inspection Nos. 57-74193, 57-87988, and 2-261476, antifading agents include those described in Japanese Patent Publication Open to Public Inspection Nos. 57-74192, 57-87989, 60-72785, 61-146591, 1-95091, and 3-13376.

The ink receiving layer may include pH modifiers, adhesion promoters, rheology modifiers, latexes, biocides, dyes, optical brighteners, whitening agents, described in Japanese Patent Publication Open to Public Inspection Nos. 59-42993, 59-52689, 62-280069, 61-242871, and 4-219266, and antistatic agents.

The ink receiving layer of the invention can contain one or more mordanting species or polymers. The mordant polymer can be a soluble polymer, a charged molecule, or a crosslinked dispersed microparticle. The mordant can be non-ionic, cationic or anionic. Examples of a mordant are polymers or copolymers containing a quaternized nitrogen moiety, such as, for example, poly(styrene-co-1-vinylimidazole-co-1-vinyl-3-benzylimidazolium chloride), poly(styrene-co-1-vinylimidazole-co-1-vinyl-3-hydroxyethyl-imidazolium chloride), poly(styrene-co-1-vinylimidazole-co-1-vinyl-3-benzylimidazolium chloride-co-1-vinyl-3-hydroxyethylimidazolium chloride), poly(vinylbenzyltrimethylammonium chloride-co-divinylbenzene), poly(ethyl acrylate-co-1-vinylimidazole-co-1-vinyl-3-benzylimidazolium chloride), or poly(styrene-co-4-vinylpyridine-co-4-hydroxyethyl-1-vinylpyridinium chloride). In a preferred embodiment of the invention, the quaternary nitrogen moiety incorporated in the polymer may be a salt of trimethylvinylbenzylammonium, benzyldimethylvinylbenzylammonium, dimethyloctadecylvinylbenzylammonium, glycidyltrimethylammonium, 1-vinyl-3-benzylimidazolium, 1-vinyl-3-hydroxyethylimidazolium or 4-hydroxyethyl-1-vinylpyridinium. Preferred counter ions which can be used include chlorides or other counter ions as disclosed in U.S. Patents 5,223,338, 5,354,813, and 5,403,955. Other mordants suitable for the invention may be cationic modified products of polymers such as poly(vinyl alcohol), gelatin, chitosan, polyvinylamine, polyethylene-imine, polydimethyldiallyl ammonium chloride, polyalkylene-polyamine dicyandiamide ammonium condensate, polyvinylpyridinium halide, polymers of (meth)acryloyl oxyalkyl quaternary ammonium salt, polymers of (meth)acrylamide alkyl quaternary ammonium salt, ω-chloro-poly(oxyethylene-polymethylene quaternary ammonium alkylate), methyl glycol chitosan, poly(vinylpyridine), propylene oxide based triamines of the Jeffamine T series, made by Texaco, Inc., quaternary acrylic copolymer latexes, phosphonium compounds, sulfonimides, sulfonated polymers and dispersed particles, and alumina hydrate. Other mordants suitable for the invention may be polymers, copolymers, or latexes containing carboxylic acid, sulfonic acid, sulfonamide, sulfonimide, or phosphonic acid, such as carboxylated and sulfonated acrylates or methacrylates, carboxylated styrene butadienes, sulfonated nylons, polyesters and polyurethanes, and their salts. In a preferred embodiment of this invention, the mordanting unit may be chemically incorporated within the chemical structure of the polyester bead. For example, a sulfonated monomer within the porous polyester structure may serve as a mordant for cationic dye species.
The ink receiving element may contain multiple individual ink receiving layers. Each being comprised of a different composition, combinations of porous organic particles with differing mean diameters, and layer thickness. For these multilayer structures, the terms as used herein, "top", "upper", and "above" mean the layer that is farther from the support in relation to the relative positioning with respect to the other layers. The terms "bottom" "lower" and "below" mean the layer that is closer to the support in relation to the relative positioning with respect to the other layers. In one embodiment, the inkjet recording element has a layer structure wherein at least one layer comprising porous polyester particles having a mean diameter of greater than 0.5 µm is located below a layer comprising porous organic particles having a mean diameter of less than 0.5 µm. In another embodiment, the inkjet recording element has a structure with at least one layer of porous polyester particles, having a mean diameter of greater than 0.5 µm in combination with porous polyester particles having a mean diameter of less than 0.5 micrometers, located below a layer comprising porous organic particles having a mean diameter of less than 0.5 µm. In another embodiment, the inkjet recording element has a structure wherein at least one layer comprising porous polyester particles having a mean diameter of greater than 0.5 µm is located below a layer comprising porous organic particles, having a mean diameter of less than 0.5 µm in combination with porous polyester particles having a mean diameter of greater than 0.5 µm. In yet another embodiment, the inkjet recording element has a structure wherein at least one layer comprising porous polyester particles, having a mean diameter of greater than 0.5 µm in combination with porous polyester particles having a mean diameter of less than 0.5 µm, is located below a layer comprising porous organic particles, having a mean diameter of less than 0.5 µm in combination with porous polyester particles having a mean diameter of greater than 0.5 µm.

The total thickness of the ink receiving layer(s) may range from 5 to 100 µm, preferably from 10 to 50 µm. The coating thickness required is determined through the need for the coating to act as a sump for absorption of ink solvent and the need to hold the ink near the coating surface. In a multilayer structure, the ink receiving layer containing porous organic particles having a mean diameter of less than 0.5 µm has a preferred thickness of from 1 to 20 µm. The inkjet recording element containing porous organic, especially polyester, particles having a mean diameter of greater than 0.5 µm has a preferred thickness of from 5 to 50 µm. The ink receiving layers have a preferred combined thickness of from 6 to 65 µm. In one embodiment of the invention, the inkjet recording element demonstrates improved ozone resistance when the element further comprises absorbed copper phthalocyanine dye, thereby having a dye density loss in ozone of less then 2 % per day per ppm ozone. When, the inkjet recording element is prepared as single layer, gloss improvements become most easily measurable and the element preferably demonstrates a surface gloss of greater than or equal to 20 at 60 degrees.

In addition to the ink receiving layer, the recording element may also contain a base layer, next to the support, the function of which is to absorb the solvent from the ink. Materials useful for this layer include inorganic particles and polymeric binder, or highly swellable polymers such as gelatin.

The support for the inkjet recording element used in the invention can be any of those usually used for inkjet receivers. The support can be either transparent or opaque. Opaque supports include plain paper, coated paper, resin-coated paper such as polyolefin-coated paper, synthetic paper, photographic paper support, melt-extrusion-coated paper, and polyolefin-laminated paper, such as biaxially oriented support laminates. Biaxially oriented support laminates are described in U.S. Patents 5,853,965, 5,866,282, 5,874,205, 5,888,643, 5,888,681, 5,888,683, and 5,888,714. These biaxially oriented supports include a paper base and a biaxially oriented polyolefin sheet, typically polypropylene, laminated to one or both sides of the paper base. The support can also consist of microporous materials such as polyethylene polymer-containing material sold by PPG Industries, Inc., Pittsburgh, Pennsylvania under the trade name of Teslin®, Tyvek® synthetic paper (DuPont Corp.), impregnated paper such as Duraform®, and OPPalyte® films (Mobil Chemical Co.) and other composite films listed in U.S. Patent 5,244,861. Transparent supports include glass, cellulose derivatives, such as a cellulose ester, cellulose triacetate, cellulose diacetate, cellulose acetate propionate, cellulose acetate butyrate, polyesters, such as poly(ethylene terephthalate), poly(ethylene naphthalate), poly-1,4-cyclohexanedimethylene terephthalate, poly(butylene terephthalate), and copolymers thereof, polyimides, polyamides, polycarbonates, polystyrene, polyolefins, such as polyethylene or polypropylene, polysulfones, polyacrylates, polyether imides, and mixtures thereof. The papers listed above include a broad range of papers, from high end papers, such as photographic paper to low end papers, such as newsprint. In a preferred embodiment, Ektacolor paper made by Eastman Kodak Co. is employed. The term as used herein, "transparent" means the ability to pass radiation without significant deviation or absorption.

The support used in the invention may have a thickness of from 50 to 500 µm, preferably from 75 to 300 µm. Antioxidants, brightening agents, antistatic agents, plasticizers and other known additives may be incorporated into the support, if desired.

In order to improve the adhesion of the ink receiving layer to the support, an under-coating or subbing layer may be applied to the surface of the support. This layer may be an adhesive layer such as, for example, halogenated phenols, partially hydrolyzed vinyl chloride-co-vinyl acetate polymer, vinylidene chloride-methyl acrylate-itaconic acid terpolymer, a vinylidene chloride-acrylonitrile-acrylic acid terpolymer, or a glycidyl (meth)acrylate polymer or copolymer. Other chemical adhesives, such as polymers, copolymers, reactive polymers or copolymers, that exhibit good bonding between the ink receiving layer and the support can be used. The polymeric binder in the subbing layer employed in the invention is preferably a water soluble or water dispersible polymer such as poly(vinyl alcohol), poly(vinyl pyrrolidone), gelatin, a cellulose ether, a poly(oxazoline), a poly(vinylacetamide), partially hydrolyzed poly(vinyl acetate/vinyl alcohol), poly(acrylic acid), poly(acrylamide), poly(alkylene oxide), a sulfonated or phosphated polyester or polystyrene, casein, zein, albumin, chitin, chitosan, dextran, pectin, a collagen derivative, collodian, agar-agar, arrowroot, guar, carrageenan, tragacanth, xanthan, rhamsan, a latex such as poly(styrene-co-butadiene), a polyurethane latex, a polyester latex, or a poly(acrylate), poly(methacrylate), poly(acrylamide) or copolymers thereof.

In a preferred embodiment, the subbing layer polymeric binder is a sulfonated polyester dispersion, such as AQ29 ® (Eastman Chemical Co.), gelatin, a polyurethane or poly(vinyl pyrrolidone). The polymeric binder for the subbing layer is preferably used in an amount of from 1 to 50 g/m², preferably from 1 to 20 g/m².

A borate or borate derivative employed in the subbing layer of the ink jet recording element of the invention may be, for example, borax, sodium tetraborate, boric acid, phenyl boronic acid, or butyl boronic acid. As noted above, the borate or borate derivative may be used in an amount of from 3 to 50 g/m², preferably from 3 to 10 g/m². It is believed that upon coating, the borate or borate derivative in the subbing layer diffuses into the image-receiving layer to cross-link the cross-linkable binder in the image-receiving layer.

Other methods to improve the adhesion of the layer to the support include surface treatment of the support by corona-discharge, plasma-treatment in a variety of atmospheres, UV treatment, which may be performed prior to applying the layer to the support.

The recording element of the invention can contain one or more conducting layers such as an antistatic layer to prevent undesirable static discharges during manufacture and printing of the image. This may be added to either side of the element. Antistatic layers conventionally used for color films have been found to be satisfactory, such as those in U.S. Patent 5,147,768. Preferred antistatic agents include mental oxides, e.g., tin oxide, antimony doped tin oxide and vanadium pentoxide. These antistatic agents may be preferably dispersed in a film-forming binder.

The layers described above may be coated by conventional coating means onto a support material commonly used in this art. Coating methods may include, but are not limited to, wound wire rod coating, knife coating, slot coating, slide hopper coating, gravure coating, spin coating, dip coating, skim-pan-air-knife coating, multilayer slide bead, doctor blade coating, gravure coating, reverse-roll coating, curtain coating, multilayer curtain coating. Some of these methods allow for simultaneous coatings of more than one layer, which may be preferred from a manufacturing economic perspective if more than one layer or type of layer needs to be applied. Known coating and drying methods are described in further detail in Research Disclosure no. 308119, published Dec. 1989, pages 1007 to 1008. Slide coating may be preferred, in which several layers may be simultaneously applied. The support may be stationary, or may be moving so that the coated layer may be immediately drawn into drying chambers. After coating, the layers may be generally dried by simple evaporation, which may be accelerated by known techniques such as convection heating.

The coating composition may be applied to one or both substrate surfaces through conventional pre-metered or post-metered coating methods listed above. The choice of coating process would be determined from the economics of the operation and in turn, would determine the formulation specifications such as coating solids, coating viscosity, and coating speed. After coating, the inkjet recording element may be subject to calendering or supercalendering to enhance surface smoothness. In a preferred embodiment of the invention, the inkjet recording element is subject to hot soft-nip calendering at a temperature of 65 °C and a pressure of 14000 kg/m at a speed of from 0.15 m/s to 0.3 m/s.

Inks used to image the recording elements of the present invention are well known in the art. The ink compositions used in inkjet printing typically may be liquid compositions comprising a solvent or carrier liquid, dyes or pigments, humectants, organic solvents, detergents, thickeners, preservatives. The solvent or carrier liquid can be solely water or can be water mixed with other water-miscible solvents such as polyhydric alcohols. Inks in which organic materials such as polyhydric alcohols may be the predominant carrier or solvent liquid may also be used. Particularly useful may be mixed solvents of water and polyhydric alcohols. The dyes used in such compositions may be typically water-soluble direct or acid type dyes. Such liquid compositions have been described extensively in the prior art including, for example, U.S. Patents 4,381,946, 4,239,543 and 4,781,758.

When used as inkjet imaging media, the media typically comprise a substrate or a support material having on at least one surface thereof an ink-receiving or recording or image-forming layer. If desired, in order to improve the adhesion of the ink receiving or recording layer to the support, the surface of the support may be corona-discharge-treated prior to applying the solvent-absorbing layer to the support or, alternatively, an undercoating, such as a layer formed from a halogenated phenol or a partially hydrolyzed vinyl chloride-vinyl acetate copolymer, can be applied to the surface of the support. The ink receiving or recording layer is preferably coated onto the support layer from water or water-alcohol solutions at a dry thickness ranging from 3 to 75 µm, preferably 8 to 50 µm.

Any known ink receiving layer can be used in combination with other particulate materials. For example, the ink receiving or recording layer may consist primarily of inorganic oxide particles such as silicas, modified silicas, clays, aluminas, fusible beads such as beads comprised of thermoplastic or thermosetting polymers, non-fusible organic beads, or hydrophilic polymers such as naturally-occurring hydrophilic colloids and gums such as gelatin, albumin, guar, xantham, acacia, chitosan, starches and their derivatives, derivatives of natural polymers such as functionalized proteins, functionalized gums and starches, and cellulose ethers and their derivatives, and synthetic polymers such as polyvinyloxazoline, polyvinylmethyloxazoline, polyoxides, polyethers, poly(ethylene imine), poly(acrylic acid), poly(methacrylic acid), n-vinyl amides including polyacrylamide and polyvinylpyrrolidone, and poly(vinyl alcohol), its derivatives and copolymers, and combinations of these materials. Hydrophilic polymers, inorganic oxide particles, and organic beads may be present in one or more layers on the substrate and in various combinations within a layer.

A porous structure may be introduced into ink receiving or recording layers comprised of hydrophilic polymers by the addition of ceramic or hard polymeric particulates, by foaming or blowing during coating, or by inducing phase separation in the layer through introduction of non-solvent. In general, it is preferred for the base layer to be hydrophilic, but not porous. This may be especially true for photographic quality prints, in which porosity may cause a loss in gloss. In particular, the ink receiving or recording layer may consist of any hydrophilic polymer or combination of polymers with or without additives as is well known in the art.

If desired, the ink receiving or recording layer can be overcoated with an ink-permeable, anti-tack protective layer such as, for example, a layer comprising a cellulose derivative or a cationically-modified cellulose derivative or mixtures thereof. An especially preferred overcoat is poly (1,4-anhydro-glucose-g-oxyethylene-g-(2'-hydroxypropyl)-N,N-dimethyl-N-dodecylammonium chloride). The overcoat layer is non porous, but is ink permeable and serves to improve the optical density of the images printed on the element with water-based inks. The overcoat layer can also protect the ink receiving or recording layer from abrasion, smudging, and water damage. In general, this overcoat layer may be present at a dry thickness of 0.1 to 5 µm, preferably 0.25 to 3 µm.

In practice, various additives may be employed in the ink receiving or recording layer and overcoat. These additives include surface active agents such as surfactant(s) to improve coatability and to adjust the surface tension of the dried coating, acid or base to control the pH, antistatic agents, suspending agents, antioxidants, hardening agents to cross-link the coating, antioxidants, UV stabilizers, light stabilizers, and thickeners. In addition, a mordant may be added in small quantities (2%-10% by weight of the base layer) to improve waterfastness. Useful mordants are disclosed in U.S. Patent No. 5,474,843.

The layers described above, including the ink receiving or recording layer and the overcoat layer, may be coated by conventional coating means onto a transparent or opaque support material commonly used in this art. Coating methods may include, but are not limited to, blade coating, wound wire rod coating, slot coating, slide hopper coating, gravure, curtain coating. Some of these methods allow for simultaneous coatings of both layers, which is preferred from a manufacturing economic perspective.

The IRL (ink or dye receiving layer) may be coated over a tie layer (TL). There are many known formulations, which may be useful as ink or dye receiving or recording layers. The primary requirement is that the IRL may be compatible with the inks which it will be imaged so as to yield the desirable color gamut and density. As the ink drops pass through the IRL, the ink or dyes may be retained or mordanted in the IRL, while the ink solvents pass freely through the IRL and may be rapidly absorbed by the TL. Additionally, the IRL formulation may be preferably coated from water, exhibits adequate adhesion to the TL, and allows for easy control of the surface gloss.

For example, Misuda et al in US Patents 4,879,166, 5,264,275, 5,104,730, 4,879,166, and Japanese Patents 1,095,091, 2,276,671, 2,276,670, 4,267,180, 5,024,335, and 5,016,517 disclose aqueous based IRL formulations comprising mixtures of psuedo-bohemite and certain water soluble resins. Light in US Patents 4,903,040, 4,930,041, 5,084,338, 5,126,194, 5,126,195, and 5,147,717 discloses aqueous-based IRL formulations comprising mixtures of vinyl pyrrolidone polymers and certain water-dispersible and/or water-soluble polyesters, along with other polymers and addenda. Butters et al in US Patents 4,857,386 and 5,102,717 disclose ink-absorbent resin layers comprising mixtures of vinyl pyrrolidone polymers and acrylic or methacrylic polymers. Sato et al in US Patent 5,194,317 and Higuma et al in US Patent 5,059,983 disclose aqueous-coatable IRL formulations based on poly(vinyl alcohol). Iqbal in US Patent 5,208,092 discloses water-based IRL formulations comprising vinyl copolymers, which may be subsequently cross-linked. In addition to these examples, there may be other known or contemplated IRL formulations, which are consistent with the aforementioned primary and secondary requirements of the IRL, all of which fall under the spirit and scope of the current invention.

The IRL may also contain varying levels and sizes of matting agents for the purpose of controlling gloss, friction, and/or fingerprint resistance, surfactants to enhance surface uniformity and to adjust the surface tension of the dried coating, mordanting agents, antioxidants, UV absorbing compounds, light stabilizers.

It may also be desirable to overcoat the IRL for the purpose of enhancing the durability of the imaged element. Such overcoats may be applied to the IRL either before or after the element is imaged. For example, the IRL can be overcoated with an ink-permeable layer through which inks freely pass. Layers of this type are described in US Patents 4,686,118, 5,027,131, and 5,102,717. Alternatively, an overcoat may be added after the element is imaged. Any of the known laminating films and equipment may be used for this purpose. The inks used in the aforementioned imaging process are well known, and the ink formulations are often closely tied to the specific processes, i.e., continuous, piezoelectric, or thermal. Therefore, depending on the specific ink process, the inks may contain widely differing amounts and combinations of solvents, colorants, preservatives, surfactants, humectants. Inks preferred for use in combination with the image recording elements of the present invention are water-based. However, it may be intended that alternative embodiments of the image-recording elements as described above, which may be formulated for use with inks which may be specific to a given ink-recording process or to a given commercial vendor, fall within the scope of the present invention.

Although the recording elements disclosed herein have been referred to primarily as being useful for inkjet printers, they also can be used as recording media for pen plotter assemblies. Pen plotters operate by writing directly on the surface of a recording medium using a pen consisting of a bundle of capillary tubes in contact with an ink reservoir.

The following examples are intended to further illustrate, but not to limit, the invention.

### EXAMPLES

### Preparation of porous polyester particles PE-1 through PE-10

Precursor polyesters PP-1 through PP-5 were all synthesized by a 2-stage melt polycondensation process. The chemical compositions are listed in Table 1 and the reaction times and final molecular weights are listed in Table 2. The SIP, CHDM, dibutylstannoic acid, zinc acetate, and sodium acetate were combined in a 500 ml 3-neck flask equipped with a stainless steel stirring rod, nitrogen inlet, and an arm leading to a dry ice/acetone condenser with an outlet connected to a controlled vacuum system. A graduated cylinder was connected beneath the condenser with a ground glass joint to collect and measure distillate. The reaction was heated in thermostatted bath containing a metal heating alloy. A steady stream of nitrogen was passed over the reaction mixture for 10 minutes, and was then reduced to a slightly positive flow. The temperature was held at 210-230°C for 100-250 minutes with stirring at ∼100 RPM until a clear prepolymer resulted and the calculated amount of methanol distillate had been collected in a graduated cylinder. The reaction was removed from the bath and allowed to cool. The FA and IPA were then added and the condenser was filled with ice. The reaction was restarted at 220°C and within 20 minutes water condensate began to collect. The reaction was held at 220°C for 130-460 minutes until the viscosity of the melt had increased to the point where the precursor polyester could no longer be effectively stirred and the reaction was terminated.

**Table 1**

| | **FA (g)** | **SIP (g)** | **IPA (g)** | **Mol ratio FA:SIP:IPA** | **CHDM (g)** | **Zn(OAc)₂ (g)** | **BuSn(OH)₃ (g)** | **NaOAc (g)** |
|---|---|---|---|---|---|---|---|---|
| PP-1 | 19.59 | 50.01 | - | 1:1:0 | 45.57 | 0.02 | 0.02 | 0.69 |
| PP-2 | 21.43 | 27.35 | 15.34 | 2:1:1 | 51.13 | 0.02 | 0.02 | 0.38 |
| PP-3 | 22.49 | 14.35 | 24.14 | 4:1:3 | 53.76 | 0.02 | 0.02 | 0.20 |
| PP-4 | 20.49 | 39.23 | 7.33 | 4:3:1 | 48.80 | 0.02 | 0.20 | 0.54 |
| PP-5 | 48.99 | 125.02 | - | 1:1:0 | 116.42 | 0.06 | 0.04 | 1.73 |

| | | | | | | | | |
|---|---|---|---|---|---|---|---|---|
| FA is fumaric acid SIP is dimethyl 5-sulfoisophthalate, sodium salt IPA is isophthalic acid CHDM is 1,4-cyclohexanedimethanol, mixture of *cis* and *trans* isomers. | | | | | | | | |

**Table 2**

| | **Stage 1 reaction time** | **Stage 2 reaction time** | **Mn** | **Mw** |
|---|---|---|---|---|
| PP-1 | 120 min | 130 min | 2,710 | 10,500 |
| PP-2 | 100 min | 420 min | 3,570 | 15,800 |
| PP-3 | 100 min | 460 min | 3,380 | 28,000 |
| PP-4 | 120 min | 180 min | 3,130 | 7,340 |
| PP-5 | 250 min | 200 min | 3,240 | 7,330 |

Precursor polyester PP-6 was synthesized using the same apparatus as used in the preparation of PP-1 through PP-5, and a similar 2-stage procedure. In the first stage, SIP (82.41 g, 0.28 mol), hydroquinone-bis-hydroxyethyl ether (HQBHE) (110.29 g, 0.56 mol), sodium acetate (2.28 g), and titanium isopropoxide (4 drops) were combined in a 500 ml 3-neck round bottom flask and heated for 220-240°C for 70 minutes at which point a clear, slightly orange prepolymer had formed and the calculated amount of methanol condensate had been collected. The reaction was then cooled and diethyl fumarate (47.90 g, 0.28 mol) was added. The reaction was restarted and was heated at 200°C for 100 minutes followed by 120 minutes at 220°C. A vacuum was then initiated which ramped from ambient pressure to 20 torr over 2 minutes. The viscosity of the melt began to rapidly increase and the reaction was terminated. (Mn = 2940, Mw = 5440).

Polyester beads PE-1 through PE-10 were all synthesized by the following procedure. An aqueous phase was prepared by dispersing appropriate precursor polyester in the amount of water noted in Table 3. The water generally had to be heated to 40-60°C and it required from 20 minutes to 16 hours for the precursor polyester to completely disperse, depending on the amount of SIP monomer in the precursor polyester. The aqueous phase was filtered through cheesecloth and combined in a beaker with an organic phase consisting of the toluene, DVB, hexadecane, and AIBN. The 2 phases were emulsified by any of the three methods listed in Table 3 and transferred to an appropriately sized 3-neck round bottom flask (1 L for PE-1 through 8 or 2 L for PE-9 through 10) fitted with a mechanical stirrer and a reflux condenser with nitrogen inlet. The opaque white microsuspensions were bubble degassed with nitrogen for 10 minutes, then heated overnight at 70°C for 16 hours. The resulting particle dispersions were cooled to room temperature and the toluene was removed as a water azeotrope via rotary evaporation. The dispersions were washed with 4-6 volumes of water and concentrated to 9-25% solids using a Millipore Amicon ultrafiltration system with a 100K cutoff spiral-wound dialysis cartridge. The exact concentrations of each PE dispersion are listed in Table 4.

**Table 3**

| **Disper sion** | **Precursor polyester** | **Precursor polyester (g)** | **Water (ml)** | **DVB¹ (g)** | **Toluene (g)** | **AIBN ⁵ (g)** | **Hexadecane (ml)** | **Emulsification method** |
|---|---|---|---|---|---|---|---|---|
| PE-1 | PP-1 | 20.00 | 240 | 20.00 | 40.00 | 0.40 | 4.14 | M² |
| PE-2 | PP-2 | 20.00 | 240 | 20.00 | 40.00 | 0.40 | 4.14 | M² |
| PE-3 | PP-3 | 20.00 | 240 | 20.00 | 40.00 | 0.40 | 4.14 | M² |
| PE-4 | PP-4 | 20.00 | 240 | 20.00 | 40.00 | 0.40 | 4.14 | S³ |
| PE-5 | PP-2 | 20.00 | 240 | 20.00 | 40.00 | 0.40 | 4.14 | S³ |
| PE-6 | PP-3 | 20.00 | 240 | 20.00 | 40.00 | 0.40 | 4.14 | S³ |
| PE-7 | PP-1 | 20.00 | 240 | 20.00 | 40.00 | 0.40 | 4.14 | H⁴ |
| PE-8 | PP-3 | 20.00 | 240 | 20.00 | 40.00 | 0.40 | 4.14 | H⁴ |
| PE-9 | PP-5 | 62.50 | 750 | 68.38 | 125.00 | 1.25 | 12.94 | H⁴ |
| PE-10 | PP-6 | 40.00 | 514 | 40.0 | 80.0 | 0.80 | 2.82 | H⁴ |

| | | | | | | | | |
|---|---|---|---|---|---|---|---|---|
| ¹ DVB is divinylbenzene (80% w/w with remainder being ethylstyrene, mixture of *m* and *p* isomers.) ² Reaction mixture was passed twice through an M-110T Microfluidizer (sold by Microfluidics). ³ Reaction mixture was homogenized for 10 minutes using a Silverson L4R mixer at the highest speed setting and then sonicated using a Vibra Cell probe sonicator (Sonics & Materials Inc).. ⁴ Reaction mixture was homogenized using a Silverson L4R mixer at the highest speed setting for 10 minutes. ⁵ AIBN is 2,2'-azobis(isobutyronitrile) | | | | | | | | |

### Determination of particle size and particle size distribution

The particle size and particle size distribution of each PE-1 through PE-10 was measured using a laser scattering particle size distribution analyzer, Horiba LA-920, manufactured by Horiba LTD. The results are in Table 4.

**Table 4**

| **PE dispersion** | **Wt % solids** | **Mode 1** | | | **Mode 2** | | |
|---|---|---|---|---|---|---|---|
| | | **Mean diameter (micron)** | **Proportion (%)** | **CV (%)** | **Mean diameter (micron)** | **Proportion (%)** | **CV %** |
| PE-1 | 13.54 | 0.356 | 100 | 35.2 | -- | -- | -- |
| PE-2 | 12.97 | 0.181 | 5.9 | 15.9 | 0.351 | 94.1 | 36.8 |
| PE-3 | 14.01 | 0.390 | 88.2 | 41.9 | 2.70 | 11.8 | 38.1 |
| PE-4 | 14.37 | 0.470 | 58.6 | 55.3 | 2.24 | 41.4 | 25.2 |
| PE-5 | 12.38 | 0.174 | 45.1 | 21.9 | 0.391 | 54.9 | 31.9 |
| PE-6 | 15.50 | 0.430 | 82.1 | 42.2 | 5.86 | 17.9 | 54.0 |
| PE-7 | 14.00 | 0.897 | 10.6 | 27.1 | 2.62 | 89.4 | 36.0 |
| PE-8 | 16.24 | 0.682 | 7.6 | 36.4 | 3.10 | 92.4 | 37.3 |
| PE-9 | 22.86 | 1.082 | 9.1 | 44.2 | 2.69 | 90.9 | 27.1 |
| PE-10 | 17.60 | 0.434 | 27.6 | 45.3 | 4.46 | 72.4 | 57.5 |

### 3-step Preparation of Porous Beads Containing Polyester-carbonate (PEC-1)

Polyester-diol prepolymer: Fumaric acid (100.00 g, 6.61x10⁻¹ mol), cyclohexanedimethanol (174.04 g, 1.20 mol), and Fascat 4100 (∼ 10 mg, catalytic) were combined in a 500 ml single neck round bottom flask outfitted with a mechanical stirrer and a side arm leading to a condenser assembly with a graduated cylinder to measure the volume of condensate. The reaction was placed in a bath filled with a low melting heating alloy and the temperature was ramped from 150°C to 220°C over 50 minutes then held at 220°C for 200 minutes at which point ∼32 ml of condensate had been collected. The molten polyester was cooled to room temperature, frozen in liquid nitrogen, broken up with a hammer and dried in a vacuum oven overnight at 60°C. The alcohol end groups were determined by dissolving the polyester in deuterochloroform, endcapping the polyester with trifluoroacetylimidazole, integrating the ¹⁹F NMR end group peaks, and normalizing to an internal standard. The determined value of 2.28 meq ROH/g polymer corresponds to a number average molecular weight of 877.19 g/mol.

Unsaturated polyester-carbonate: The unsaturated polyester diol oligomer from the previous step (43.85 g, 0.05 mol) and trimethylamine (22.26 g, 0.22 mol) were dissolved in dichloromethane (150 g). While stirring at room temperature, a solution of bisphenol A bis(chloroformate) (47.66 g, 0.05 g) in dichloromethane (50 ml) was slowly added over ∼20 min. The reaction was allowed to proceed at room temperature for two hours, by which time it had become notably viscous and was further diluted 100 g dichloromethane. The product solution was then extracted once with 250 ml of 2% hydrochloric acid, and twice with water. The product solution was precipitated into methanol and dried overnight in a vacuum oven at 60°C. Analysis by Differential scanning calorimetry showed a Tg of 89.4°C. Size exclusion chromatography in hexafluoroisopropanol showed Mn = 1,390 and Mw = 80,700. The broad curve suggested that the polymer may be highly branched.

Particles containing polyester-co-carbonate: An organic phase was prepared consisting of the unsaturated polyester-co-carbonate from the previous step (10.00 g) toluene (20.00 g), chloromethylstyrene (5.00 g), 80% divinylbenzene (5.00g, mixture of *m* and *p* isomers with remainder being ethylstyrene), hexadecane (0.80 g), and Vazo 52® initiator (0.20 g). The components were stirred until a clear, heterogeneous solution resulted. An aqueous phase was prepared consisting of dodecanethiol-endcapped polyacrylamide decamer surfactant (1.60 g, prepared as described in US 6,127,453 column 9 lines 40-55) dissolved in deionized water (120.00). The two phases were combined and sonicated using a Vibra Cell ® probe sonicator (Sonics & Materials Inc.) at the highest power setting for 10 minutes, then transferred to a 500 ml 3-neck round bottomed flask outfitted with a condenser, nitrogen inlet, and mechanical stirrer. The reaction mixture was bubble degassed with nitrogen for 10 minutes and heated for 16 hours with vigorous stirring at 60°C in a thermostatted water bath. The toluene was then removed via rotary evaporation and dimethylethanolamine (1.17 g) was added. The quaternization reaction was allowed to proceed at 60°C for 16 hours and the excess amine and surfactant was removed via dialysis using 12-14K cutoff cellulose dialysis tubing for 16 hours to yield a product dispersion of 13.3% solids. Analysis of the product dispersion using a Horiba® LA-920 particle sizing instrument showed a bimodal distribution with a mean particle diameter of 1.462 µm, a major mode at 0.36 µm, and a smaller mode, presumably due to secondary aggregation, at ∼6 µm.

### 2-step Preparation of Bead Containing Polyester-urethane (PEU-1).

Polyester-diol prepolymer: This reaction was set up and run in an identical manner as that described in step 1 of the preparation of PEC-1 using Maleic anhydride (107.61 g, 1.10 mol), neopentyl glycol (137.15 g, 1.32 mol), and Fascat 4100 (∼ 5 mg, catalytic). The alcohol end groups were determined by direct quantification using 1 H NMR with an internal standard. The determined value of 2.0 meq ROH/g polymer corresponds to a number average molecular weight of 1036.3 g/mol.

Particles containing polyester-urethane: An organic phase was prepared consisting of the polyester-diol oligomer from the previous step (10.00 g) toluene (55.20 g), Desmodur N3300® triisocyanate resin (3.80 g), stannous octanoate (0.05 g), dibutyltin dilaurate (0.05 g), 80% divinylbenzene (41.40g, mixture of *m* and *p* isomers with remainder being ethyl styrene), hexadecane (2.21 g), and AIBN initiator (1.03 g). The components were stirred until a clear, heterogeneous solution resulted. An aqueous phase was prepared consisting of sodium dodecylsulfate (4.40 g) dissolved in deionized water (120.00). The two phases were combined and emulsified using a Silverson L4R mixer at the highest speed for 10 minutes followed by passage twice through an M-110T Microfluidizer® (sold by Microfluidics). The resulting emulsion was poured into a 3-neck 2000 ml round bottom flask outfitted with a mechanical stirrer, condenser, and nitrogen inlet and was bubble degassed with nitrogen for 10 minutes. The emulsion was heated for 16 hours with vigorous stirring in a thermostatted water bath at 70°C and the toluene was removed via rotary evaporation. The resulting particle dispersion had 10.23% solids. Analysis of the product dispersion using a Horiba® LA-920 particle sizing instrument showed a single mode with a mean particle diameter of 0.153 µm.

### Preparation of Element 1

A coating composition was prepared from 62.78 wt. % of dispersion PE-1, 1.5 wt. % poly(vinyl alcohol), PVA, (Gohsenol® GH-17 from Nippon Gohsei Co.), and 35.72 wt. % water. [The relative proportions of porous polyester particle to PVA are therefore 85/15 by weight]. The coating composition was coated onto a base support comprised of a polyethylene resin coated photographic paper stock, which had been previously subjected to corona discharge treatment, using a calibrated coating knife, and dried to remove substantially all solvent components to form the ink receiving layer. The thickness of the dry ink receiving layer was measured to be about 17 ± 2 µm. The measured surface gloss at 60 degrees was 36 and the ink dry time was measured to be less than 10 seconds.

### Preparation of Element 2

A coating composition was prepared from 61.68 wt. % of dispersion PE-2, 2.0 wt. % poly(vinyl alcohol), PVA, (Gohsenol® GH-17 from Nippon Gohsei Co.), and 36.32 wt. % water. [The relative proportions of porous polyester particle to PVA are therefore 80/20 by weight]. The coating composition was coated and dried the same as Element 1. The thickness of the dry ink receiving layer was measured to be about 19 ± 2 µm.

### Preparation of Element 3

A coating composition was prepared from 57.10 wt. % of dispersion PE-3, 2.0 wt. % poly(vinyl alcohol), PVA, (Gohsenol® GH-17 from Nippon Gohsei Co.), and 40.90 wt. % water. [The relative proportions of porous polyester particle to PVA are therefore 80/20 by weight]. The coating composition was coated and dried the same as Element 1. The thickness of the dry ink receiving layer was measured to be about 46 ± 2 µm.

### Preparation of Element 4

A coating composition was prepared from 59.15 wt. % of dispersion PE-4, 1.5 wt. % poly(vinyl alcohol), PVA, (Gohsenol® GH-17 from Nippon Gohsei Co.), and 39.35 wt. % water. [The relative proportions of porous polyester particle to PVA are therefore 85/15 by weight]. The coating composition was coated and dried the same as Element 1. The thickness of the dry ink receiving layer was measured to be about 18 ± 2 µm.

### Preparation of Element 5

A coating composition was prepared from 64.62 wt. % of dispersion PE-5, 2.0 wt. % poly(vinyl alcohol), PVA, (Gohsenol® GH-17 from Nippon Gohsei Co.), and 33.38 wt. % water. [The relative proportions of porous polyester particle to PVA are therefore 80/20 by weight]. The coating composition was coated and dried the same as Element 1. The thickness of the dry ink receiving layer was measured to be about 25 ± 2 µm.

### Preparation of Element 6

A coating composition was prepared from 51.61 wt. % of dispersion PE-6, 2.0 wt. % poly(vinyl alcohol), PVA, (Gohsenol® GH-17 from Nippon Gohsei Co.), and 46.39 wt. % water. [The relative proportions of porous polyester particle to PVA are therefore 80/20 by weight]. The coating composition was coated and dried the same as Element 1. The thickness of the dry ink receiving layer was measured to be about 24 ± 2 µm.

### Preparation of Control Element C-1

A coating composition was prepared from 60.71 wt. % of dispersion PE-7, 1.5 wt. % poly(vinyl alcohol), PVA, (Gohsenol® GH-17 from Nippon Gohsei Co.), and 37.79 wt. % water. [The relative proportions of porous polyester particle to PVA are therefore 85/15 by weight]. The coating composition was coated and dried the same as Element 1. The thickness of the dry ink receiving layer was measured to be about 26 ± 2 µm.

### Preparation of Control Element C-2

A coating composition was prepared from 52.34 wt. % of dispersion PE-8, 1.5 wt. % poly(vinyl alcohol), PVA, (Gohsenol® GH-17 from Nippon Gohsei Co.), and 46.16 wt. % water. [The relative proportions of porous polyester particle to PVA are therefore 85/15 by weight]. The coating composition was coated and dried the same as Element 1. The thickness of the dry ink receiving layer was measured to be about 32 ± 2 µm.

### Preparation of Control Element C-3

Control Element C-3 was a commercially available inkjet non-porous receiver paper containing a high amount of gelatin, "Kodak Inkjet Photo Paper", catalogue No. 1181197 from Eastman Kodak Company.

### Preparation of Control Element C-4

Control Element C-4 was a commercially available inkjet porous receiver paper containing a high amount of silica fine particles, "Epson Premium Glossy Photo Paper", catalogue No. 5041286 from Epson.

### Printing and dye stability testing

The above elements and control elements of Example 1 were printed using a Lexmark Z51 inkjet printer and a cyan inkjet ink, prepared using a standard formulation with a copper phthalocyanine dye (Clariant Direct Turquoise Blue FRL-SF). The red channel density (cyan) patches at D-max (the highest density setting) were read using an X-Rite ® 820 densitometer. The cyan density is reported in Table 5. The printed elements were then subjected to 4 days exposure to a nitrogen flow containing 5 ppm ozone. The density of each patch was read after the exposure test using an X-Rite ® 820 densitometer. The % dye retention was calculated as the ratio of the density after the exposure test to the density before the exposure test. The results for cyan D-max are reported in Table 5.

### Surface gloss measurement

The gloss of the top surface of the unprinted ink receiving layer was measured using a BYK Gardner gloss meter at an angle of illumination/reflection of 60°. The results are related to a highly polished black glass with a refractive index of 1.567 that has a specular gloss value of 100. The results are reported in Table 5.

### Measurement of ink dry time:

A drop (from a 10 microliter capillary tube) of a magenta inkjet ink, prepared using a standard formulation with Dye 6 from U.S. Patent 6,001,161, was placed on each unprinted element and the time that it took for this spot to become dry to the touch was measured as the "ink drying time" as shown in Table 5.

**Table 5**

| **Element** | **Cyan D-max** | **% dye retention cyan D-max** | **60° gloss** | **Ink drying time (seconds)** |
|---|---|---|---|---|
| 1 | 1.6 | 91 | 36 | < 10 |
| 2 | 1.7 | 94 | 72 | 60 |
| 3 | 1.6 | 96 | 20 | < 10 |
| 4 | 1.6 | 85 | 28 | 40 |
| 5 | 1.7 | 96 | 70 | 150 |
| 6 | 1.8 | 99 | 40 | < 10 |
| Control C-1 | 1.1 | 96 | 3 | < 10 |
| Control C-2 | 1.4 | 93 | 5 | 50 |
| Control C-3 | 1.8 | 99 | 88 | > 180 |
| Control C-4 | 2.2 | 27 | 38 | 45 |

The above results show that high surface gloss for the element containing porous polyester particles can only be achieved with the incorporation of porous polyester particles that have a mean diameter of less than 0.5 µm, compared to the control elements having only porous polyester particles that have a mean diameter of greater than 0.5 µm. The above results also show that, although high surface gloss can be attained with a layer that does not contain porous polyester particles (Control element C-3), rapid ink drying time is not achieved unless the layer contains porous polyester particles. The above results also show that, although high surface gloss and rapid ink drying time can be attained with a porous layer comprising fine-particle silica (Control Element C-4), dye stability towards environmental gases remains poor.

### Example 2

### Preparation of Control Element C-5 (single layer of larger size particles)

A coating composition was prepared from 53.92 wt. % of dispersion PE-9, 2.18 wt. % poly(vinyl alcohol), PVA, (Gohsenol® GH-17 from Nippon Gohsei Co.), and 43.90 wt. % water. [The relative proportions of porous polyester particle to PVA are therefore 85/15 by weight]. The coating composition was metered to a slot-die coating apparatus and coated onto a base support comprised of a polyethylene resin coated photographic paper stock, which had been previously subjected to corona discharge treatment, moving at a speed of about 2.4 m/min. The coated support immediately entered the drying section of the coating machine to remove substantially all solvent components and form an ink receiving layer. The thickness of the dry ink receiving layer was measured to be about 15 ± 2 µm. The measured surface gloss at 60 degrees was 3 and the ink dry time was measured to be greater than 180 seconds.

### Preparation of Element 7

A coating composition (Solution S-9) was prepared the same as in Control Element C-5. A second homogeneous coating composition (Solution S-1) was prepared the same as in Element 1. Both coating compositions were metered to a multiple-slot-die coating apparatus and coated simultaneously, with Solution S-9 being located below (closer to the support than) Solution S-1, onto a base support comprised of a polyethylene resin coated photographic paper stock, which had been previously subjected to corona discharge treatment, moving at a speed of about 2.4 m/min. The coated support immediately entered the drying section of the coating machine to remove substantially all solvent components and form a two-layer image receiving element. The combined thickness of the dry ink receiving layers was measured to be about 19 ± 2 µm. The measured surface gloss at 60 degrees was 23 and the ink dry time was measured to be 100 seconds.

### Preparation of Element 8

Coating compositions S-9 and S-1 were prepared the same as Element 7 except that Solution S-1 was 59.08 wt. % of dispersion PE-1, 2.0 wt. % poly(vinyl alcohol), PVA, (Gohsenol® GH-17 from Nippon Gohsei Co.), and 38.92 wt. % water. [The relative proportions of porous polyester particle to PVA are therefore 80/20 by weight]. The coating compositions were coated and dried the same as Element 7. The combined thickness of the dry ink receiving layers was measured to be about 20 ± 2 µm. The measured surface gloss and the ink dry time are reported in Table 6.

### Preparation of Element 9

A coating composition (Solution S-9) was prepared the same as in Control Element C-5. A second homogeneous coating composition (Solution S-2) was prepared the same as in Element 2 except that Solution S-2 was prepared from 65.54 wt. % of dispersion PE-2, 1.5 wt. % poly(vinyl alcohol), PVA, (Gohsenol® GH-17 from Nippon Gohsei Co.), and 32.96 wt. % water. [The relative proportions of porous polyester particle to PVA are therefore 85/15 by weight]. The coating compositions were coated and dried the same as Element 7, with Solution S-9 being located below (closer to the support than) Solution S-2. The thickness of the dry lower layer was measured to be about 12 ± 2 µm and the thickness of the dry upper layer was measured to be about 9 ± 2 µm. The measured surface gloss and the ink dry time are reported in Table 6.

### Preparation of Element 10

Coating compositions S-9 and S-2 were prepared, coated and dried the same as Element 9 except that the thickness of the layers were different. The combined thickness of the dry ink receiving layers was measured to be about 12 ± 2 µm. The measured surface gloss and the ink dry time are reported in Table 6.

### Preparation of Element 11

A coating composition (Solution S-9) was prepared the same as in Control Element C-5. A second homogeneous coating composition (Solution S-10) was prepared from 48.30 wt. % of dispersion PE-10, 1.5 wt. % poly(vinyl alcohol), PVA, (Gohsenol® GH-17 from Nippon Gohsei Co.), and 50.20 wt. % water. [The relative proportions of porous polyester particle to PVA are therefore 85/15 by weight]. The coating compositions were coated and dried the same as Element 7, with Solution S-9 being located below (closer to the support than) Solution S-10. The thickness of the dry lower layer was measured to be about 20 ± 2 µm and the thickness of the dry upper layer was measured to be about 5 ± 2 µm. The measured surface gloss and the ink dry time are reported in Table 6.

The above elements of Example 2 were printed using a Lexmark Z51 inkjet printer and a cyan inkjet ink, prepared using a standard formulation with a copper phthalocyanine dye (Clariant Direct Turquoise Blue FRL-SF). The red channel density (cyan) patches at D-max (the highest density setting) are reported in Table 6.

**Table 6**

| **Element** | **Cyan D-max** | **60° gloss** | **Ink drying time (second**s) |
|---|---|---|---|
| 7 | 1.7 | 23 | 100 |
| 8 | 1.6 | 30 | 120 |
| 9 | 1.7 | 65 | 120 |
| 10 | 1.7 | 48 | 180 |
| 11 | 1.6 | 10 | 20 |
| Control C-5 | 1.1 | 3 | > 180 |

The above results show that high surface gloss and improved print density for the element can be achieved with a multi-layer ink receiving layer structure, particularly when the upper layer contains porous polyester particles that have a mean diameter of less than 0.5 µm.

### Example 3

### Preparation of Element 12

A coating composition was prepared from 48.7 wt. % of aqueous dispersion PEU-1 (10.23 wt % solids in water), 5.0 wt. % poly(vinyl alcohol), PVA, (Gohsenol® GH-17 from Nippon Gohsei Co.), and 46.3 wt. % water. [The relative proportions of porous organic particle to PVA are therefore 50/50 by weight]. The coating composition was coated and dried the same as Element 1.

### Preparation of Element 13

A coating composition was prepared from 38.0 wt. % of aqueous dispersion PEC-1 (13.33 wt % solids in water), 5.0 wt. % poly(vinyl alcohol), PVA, (Gohsenol® GH-17 from Nippon Gohsei Co.), and 57.0 wt. % water. [The relative proportions of porous polyester particle to PVA are therefore 50/50 by weight]. The coating composition was coated and dried the same as Element 1. The thickness of the dry ink receiving layer was measured to be about 11 ± 2 µm.

The above elements of Example 3 were printed using a Lexmark Z51 inkjet printer and a cyan inkjet ink, prepared using a standard formulation with a copper phthalocyanine dye (Clariant Direct Turquoise Blue FRL-SF). The red channel density (cyan) patches at D-max (the highest density setting) were measured to be 1.5 for element 12 and 1.7 for element 13.

## Claims

1. An inkjet recording element comprising a support, at least one porous ink receiving layer comprising crosslinked porous polyester-containing particles having a mean diameter of less than 0.5 µm and having ionic groups, wherein said crosslinked porous polyester-containing particles are prepared from an unsaturated precursor condensation polymer that comprises polyester;
wherein the crosslinked porous polyester-containing particles are obtainable by crosslinking the unsaturated precursor condensation polymer within an oil-in-water emulsion in the presence of a water-immiscible solvent, wherein the crosslinking reaction is a radical initiated polymerization of an ethylenically unsaturated monomer which readily polymerizes with the unsaturated units in the unsaturated precursor condensation polymer, after which the water-immiscible organic solvent is removed to yield the porous crosslinked polyester-containing particles in a dispersion.

2. The inkjet recording element of claim 1 wherein said ethylenically unsaturated monomer is a vinyl monomer.

3. The inkjet recording element of claims 1-2 wherein said unsaturated precursor condensation polymer comprises ionic groups having quaternary ammonium moieties.

4. The inkjet recording element of claim 1 wherein said particles have an ionic group equivalent weight of from 40 to 2000 grams per mole of ionic unit.

5. The inkjet recording element of claim 1 wherein said at least one layer further comprises a polymeric binder.

6. The inkjet recording element of claim 1 wherein said particles comprise from 50 to 95% by weight of said at least one layer.

7. The inkjet recording element of claim 1 wherein the unsaturated precursor condensation polymer may comprise at least one bond selected from the group consisting of ester-co-urethane, ester-co-urea, ester-co-amide, ester-co-carbonate.

8. The inkjet recording element of claim 1 wherein the monomer is selected from the group consisting of divinylbenzene, divinyl adipate, and cyclohexanedimethanol divinyl ether.

9. The inkjet recording element of claim 1 wherein the unsaturated precursor condensation polymer comprises at least one ethylenically unsaturated polyacids selected from the group consisting of maleic, fumaric, itaconic, phenylenediacrylic, citraconic and mesaconic acid.

10. A method of forming an inkjet print comprising providing the inkjet recording element of claim 1 and printing on said inkjet recording element utilizing an inkjet printer.

## Patentansprüche

1. Tintenstrahl-Aufzeichnungselement, das Folgendes umfasst: einen Träger und wenigstens eine poröse tintenaufnehmende Schicht, die vernetzte poröse polyesterhaltige Teilchen mit einem mittleren Durchmesser von weniger als 0,5 µm und ionischen Gruppen umfasst, wobei die vernetzten porösen polyesterhaltigen Teilchen aus einem ungesättigten Vorläufer-Kondensationspolymer, das Polyester umfasst, hergestellt sind;
wobei die vernetzten porösen polyesterhaltigen Teilchen durch Vernetzen des ungesättigten Vorläufer-Kondensationspolymers innerhalb einer ÖI-in-Wasser-Emulsion in Gegenwart eines mit Wasser nicht mischbaren Lösungsmittels erhältlich sind, wobei die Vernetzungsreaktion eine radikalisch gestartete Polymerisation eines ethylenisch ungesättigten Monomers ist, das leicht mit den ungesättigten Einheiten in dem ungesättigten Vorläufer-Kondensationspolymer polymerisiert, woraufhin das mit Wasser nicht mischbare organische Lösungsmittel entfernt wird, so dass man die porösen vernetzten polyesterhaltigen Teilchen in einer Dispersion erhält.

2. Tintenstrahl-Aufzeichnungselement gemäß Anspruch 1, wobei das ethylenisch ungesättigte Monomer ein Vinylmonomer ist.

3. Tintenstrahl-Aufzeichnungselement gemäß Anspruch 1-2, wobei das ungesättigte Vorläufer-Kondensationspolymer ionische Gruppen umfasst, die quartäre Ammonium-Struktureinheiten aufweisen.

4. Tintenstrahl-Aufzeichnungselement gemäß Anspruch 1, wobei die Teilchen ein Äquivalentgewicht der ionischen Gruppen von 40 bis 2000 Gramm pro Mol der ionischen Einheit aufweisen.

5. Tintenstrahl-Aufzeichnungselement gemäß Anspruch 1, wobei die wenigstens eine Schicht weiterhin ein polymeres Bindemittel umfasst.

6. Tintenstrahl-Aufzeichnungselement gemäß Anspruch 1, wobei die Teilchen 50 bis 95 Gew.-% der wenigstens einen Schicht umfassen.

7. Tintenstrahi-Aufzeichnungselement gemäß Anspruch 1, wobei das ungesättigte Vorläufer-Kondensationspolymer wenigstens eine Bindung umfassen kann, die aus der Gruppe ausgewählt ist, die aus Ester-co-Urethan, Ester-co-Harnstoff, Ester-co-Amid und Ester-co-Carbonat besteht.

8. Tintenstrahl-Aufzeichnungselement gemäß Anspruch 1, wobei das Monomer aus der Gruppe ausgewählt ist, die aus Divinylbenzol, Divinyladipat und Cyclohexandimethanoldivinylether besteht.

9. Tintenstrahl-Aufzeichnungselement gemäß Anspruch 1, wobei das ungesättigte Vorläufer-Kondensationspolymer wenigstens eine ethylenisch ungesättigte Polysäure umfasst, die aus der Gruppe ausgewählt ist, die aus Malein-, Fumar-, Itacon-, Phenylendiacryl-, Citracon- und Mesaconsäure besteht.

10. Verfahren zur Bildung eines Tintenstrahlausdrucks, das das Bereitstellen des Tintenstrahl-Aufzeichnungselements gemäß Anspruch 1 und das Drucken auf das Tintenstrahl-Aufzeichnungselement unter Verwendung eines Tintenstrahldruckers umfasst.

## Revendications

1. Elément d'enregistrement par jet d'encre comprenant un support, au moins une couche poreuse recevant l'encre comprenant des particules poreuses réticulées contenant un polyester ayant un diamètre moyen inférieur à 0,5 µm et ayant des groupes ioniques, dans lequel lesdites particules poreuses réticulées contenant un polyester sont préparées à partir d'un polycondensat précurseur insaturé qui comprend un polyester ;
dans lequel les particules poreuses réticulées contenant un polyester peuvent être obtenues par réticulation du polycondensat précurseur insaturé dans une émulsion huile-dans-eau en présence d'un solvant non miscible à l'eau, dans lequel la réaction de réticulation est une polymérisation initiée par radical d'un monomère insaturé éthyléniquement qui se polymérise facilement avec les unités insaturées présentes dans le polycondensat précurseur insaturé, après quoi le solvant organique non miscible à l'eau est éliminé pour obtenir les particules poreuses réticulées contenant un polyester en dispersion.

2. Elément d'enregistrement par jet d'encre selon la revendication 1, dans lequel ledit monomère insaturé éthyléniquement est un monomère vinylique.

3. Elément d'enregistrement par jet d'entre selon les revendications 1-2, dans lequel ledit polycondensat précurseur insaturé comprend des groupes ioniques ayant des motifs ammonium quaternaire.

4. Elément d'enregistrement par jet d'encre selon la revendication 1, dans lequel lesdites particules ont un poids équivalent de groupes ioniques allant de 40 à 2000 grammes par mole d'unité ionique.

5. Elément d'enregistrement par jet d'encre selon la revendication 1, dans lequel ladite au moins une couche comprend de plus un liant polymère.

6. Elément d'enregistrement par jet d'encre selon la revendication 1, dans lequel lesdites particules comprennent de 50 à 95 % en poids de ladite au moins une couche.

7. Elément d'enregistrement par jet d'encre selon la revendication 1, dans lequel le polycondensat précurseur insaturé peut comprendre au moins une liaison choisie dans le groupe consistant en ester-co-uréthane, ester-co-urée, ester-co-amide, ester-co-carbonate.

8. Elément d'enregistrement par jet d'encre selon la revendication 1, dans lequel le monomère est choisi dans le groupe consistant en divinylbenzene, divinyl adipate et cyclohexanediméthanol divinyl éther.

9. Elément d'enregistrement par jet d'encre selon la revendication 1, dans lequel le polycondensat précurseur insaturé comprend au moins un polyacide insaturé éthyléniquement, choisi dans le groupe consistant en acide maléique, fumarique, itaconique, phénylènediacrylique, citraconique et mésaconique.

10. Procédé pour former une impression par jet d'encre comprenant la fourniture de l'élément d'enregistrement par jet d'encre selon la revendication 1 et l'impression sur ledit élément d'enregistrement par jet d'encre en utilisant une imprimante à jet d'encre.
